

XR 1,881,128

X 2012 W

SEARCH ROOM

Oct. 4, 1932.

A. C. PAYNE ET AL  
PROJECTION SCREEN

1,881,128

Original Filed Nov. 28, 1925

JBSTITUTE FOR MISSING OR

Fig. 1.



- gelatinous material
- liquid principle
- germicide, bactericide, fungicide, etc
- glycerine
- coloring matter
- light diffuser
- solvent for 6
- curing agent
- georgette silk

6  
428/24  
X 428/15  
X 428/14  
X 428/539  
X 428/901

Fig. 2.



- glue
- water
- sodium fluoride
- glycerine
- cobalt blue
- calcium
- borax
- copper sulphate

Fig. 3.



Fig. 4.



Arthur C. Payne and INVENTORS  
David F. Newell and  
W.M. Coffield ATTORNEY

OR/106-15R.

## UNITED STATES PATENT OFFICE

ARTHUR C. PAYNE, OF KEW GARDENS, AND DAVID F. NEWMAN, OF FREEPORT, NEW YORK, ASSIGNEES TO TRANS-LUX DAYLIGHT PICTURE SCREEN CORPORATION, OF NEW YORK, N. Y., A CORPORATION OF DELAWARE

## PROJECTION SCREEN

Application filed November 28, 1925, Serial No. 72,029. Renewed May 24, 1930.

This invention relates to screens for projecting systems in connection with moving pictures, stereopticon views, or the like, such screens being utilizable ordinarily for rear 5 projection although, under some circumstances, they may be utilized for front projection.

The principal object of the invention is to provide a translucent screen on which the 10 picture may be projected in a lighted or darkened room at the option of the operator. In screens of this type the picture is projected from the rear; that is, projected on the screen on the opposite side from the spectator, the spectator being in the path of the direct light instead of receiving the reflected light from the picture.

Another object is to provide a screen in which the light thrown by the projection 15 machine passes through the screen and gives the picture an appearance of unusual sharpness.

Another object is to provide a translucent screen which is flexible and which may be 20 readily rolled for transportation or storage, the folds of the screen not sticking to the adjacent fold when stored in a rolled condition.

Another object is to provide a screen which 25 may be adapted to varying climatic conditions, such as differences in temperatures and humidity, by merely varying the quantity of the ingredients used. Heretofore screens of this type have been made but it has been 30 found that a screen made of one material adapted to be used under one climatic condition will be wholly unsuitable if used under a different and widely varying climatic condition, so that screens for warm, humid climates would have to be made of one material 35 while screens for cold, dry climates would have to be made of other materials. By this invention the differences in temperature can 40 be easily taken care of by varying the relative quantities of ingredients used without the necessity of using other and different ingredients.

Another object of this invention is to provide 45 a screen which will not mildew when

left rolled in a damp place for a long period of time.

Another object of this invention is to provide a screen which will be ~~germinal-proof~~

In other words, this invention relates to 50 a screen which can be made adaptable for all ranges of temperature and climate and which may be rolled indefinitely without deterioration and which will also produce an image of unusual sharpness, and which can be used 55 in a lighted room as well as in a darkened one.

Other objects of the invention will appear from the following description.

This screen is an improvement on the type 60 of screen disclosed in Patent No. 1,151,502, issued to Troeger, on August 24, 1915.

A very satisfactory screen has been produced by using the following formula. The 65 portions given are by weight—

|                 | Parts |
|-----------------|-------|
| Glue            | 100   |
| Water           | 208   |
| Sodium fluoride | 4     |
| Glycerine       | 100   |
| Special formula | 80    |
| Cobalt blue     | 1.5   |

The glue and glycerine form the screen body and these materials may be any suitable character. The sodium fluoride acts as a germicide, a bactericide, fungicide, preservative or the like and, in lieu thereof, other agents having similar properties may be utilized. The cobalt blue serves as a light- 80 filtering agent and it, or equivalent material, may be utilized, if desired, to produce a screen of such character that it will be neutral or nearly so when acted upon by the light from the projector whereby a large 85 number of the usual yellow rays of the projecting light source are filtered out.

In preparing the screen, the glue may be soaked for an extended period, as from six 90 to eight hours, and then brought into solution by a slow heat and frequent stirring, the temperature, preferably, not greatly exceeding 178 degrees F. Preferably, the sodium fluoride is separately dissolved in water 95

and added to the glue before the aforesaid application of heat.

The glycerine may now be added, the mixture thereafter being thoroughly stirred and then preferably strained. While the mixture is being stirred and while maintained substantially at the same temperature as noted above, it is desirable that the special formula be added, the latter preferably having been previously strained.

Preferably, the cobalt blue coloring material is stirred in last, this material being added a few drops at a time until the proper color is reached. After the mixture has cooled some 30 or 40 degrees F., its consistency should be about that of a medium syrup at room temperature. If, on account of the type of glue used, the solution should be too thick, more of the sodium fluoride in water solution may be added. The molding operation may now follow.

The special formula is used as a diffuser or light-diffusing agent, and also serves as an atmospheric agent in the sense that the completed screen is thereby put in a condition resisting the otherwise damaging effects of the atmosphere. Preferably, the special formula is prepared as follows: to 100 parts of casein by weight is added 208 parts of water, 12.5 parts of borax, and 1 part of cupric sulphate. The method of preparing this formula is as follows:

The casein is placed in 130 parts of water and stirred until all of the casein has been moistened. The borax and cupric sulphate are dissolved with the remaining 78 parts of water and added to the casein mixture during gentle stirring of the latter. The mixture will then begin to thicken and within forty-eight hours will have become a thin smooth fluid which should be well stirred and left to ripen for a suitable period, as five days, more or less, after which it is ready for use.

The casein serves as a light-diffusing agent and the wafer requirement may vary somewhat depending upon the type thereof. Obviously, in accordance with certain phases of our invention, other light-diffusing agents may be substituted for the casein. The borax functions as a solvent for the casein.

The cupric sulphate serves primarily as an agent resisting action of the atmosphere on the completed screen; it acts in an anti-hydroscopic manner and serves to harden, dry and/or cure the screen. Therefore, the use of cupric sulphate renders the screen more moisture-resisting without materially detracting from its elasticity and flexibility. While the amount of cupric sulphate has been given as 1 part, where it is known that the screen is to be used in a tropical climate, this amount may be increased from 1 to 2 parts in order to increase the moisture-resisting properties of the screen. However, screens made in accordance with the formula as given

have been found to give extremely good results in tropics where only one part of cupric sulphate is used. Obviously, in lieu of cupric sulphate, other agents having similar properties may be utilized.

On the accompanying drawing, we have illustrated a screen-forming arrangement and on said drawing:

Figure 1 is a perspective view, partly in section, showing the matrix or table upon which the screen is supported during manufacture thereof;

Fig. 2 is a transverse, vertical sectional view of the table of Fig. 1 and showing a frame above the table with a stretched sheet thereon;

Fig. 3 is a vertical, sectional view of a portion of the screen before the sheet is embedded in the viscous screen material; and

Fig. 4 is a view corresponding with Fig. 3 showing the finished product.

As shown on the drawing, a dry sheet 1 of suitable fabric, as georgette silk, from which gum, grease and other material have been suitably removed, is stretched on a frame 2 defining an opening just large enough to fit snugly around the upright edge or wall 3 of the matrix table 4 on which the screen is to be molded.

After the matrix table has been brought to suitable temperature conditions, ordinarily above 100 degrees F., and with the screen-forming material in proper condition, and of proper temperature, preferably somewhat higher than the table temperature, said material should be poured on or applied to the table, preferably to such an extent that it slightly overflows the aforesaid wall 3, the height of which determines the thickness of the screen. The excess material should now be removed, as by a straight edge. After this operation, the molded material 7 is flush with the top surface of the aforesaid wall 3 as shown particularly in Fig. 2.

After the excess material has been removed as stated above, the sheet of silk is suitably lowered toward and into engagement with the upper surface of the material on the matrix table, care being taken to avoid entrapment of air between the silk sheet and the screen-forming material. In so doing, the frame holding the silk sheet comes into position around the bordering wall 3 of the matrix table, and thereupon the silk sheet sinks into or amalgamates with the screen-forming material. At this time, application of heat to the matrix table should be discontinued and, after a suitable cooling period, as two or three hours, has elapsed, a knife should be passed between the frame 2 and the wall 3 to sever said sheet from its frame. Thereafter, the molded screen may be removed from the matrix table in any suitable manner.

After completion of the screen as just described, the edges thereof should be suitably

bound, as by canvas strips, or equivalent, adhesively secured thereto and provided with eyelets. When the screen is installed for use, a suitable frame should be provided and the 5 screen positioned tautly therein, as by a rope passed through the eyelets and engaging the frame.

Although we have described the screen-forming material of our invention as formed 10 into a completed screen by a molding operation and utilized in connection with a fabric sheet, it shall be understood that our invention is not to be so limited since the fabric sheet may be omitted, if desired, and the 15 molding operation may be effected otherwise than as herein described.

While the invention has been described with respect to a certain particular preferred example which gives satisfactory results, it 20 will be understood by those skilled in the art after understanding the invention, that various changes and modifications may be made without departing from the spirit and scope of the invention and it is intended therefore 25 in the appended claims to cover all such changes and modifications.

What is claimed as new and desired to be secured by Letters Patent is:

1. A projection screen containing gelatinous material, glycerine and a liquid principally, a light diffusing agent, a curing agent, a germicide, and having a fibrous strengthening material incorporated therein, said light diffusing agent being substantially uniformly incorporated in the other screen-forming materials.

2. A projection screen containing glue, glycerine and a liquid principally, a light diffusing agent, a germicide substantially incapable of exercising a hardening effect on the screen, a curing agent, coloring material, and having a reinforcing material incorporated therein.

3. A projection screen composed principally of gelatinous material, glycerine and water and containing a light diffusing agent, a curing agent, and having a fibrous strengthening material incorporated therein, said light diffusing agent being substantially uniformly incorporated in the other screen-forming materials.

4. A projection screen resistant to atmospheric and climatic conditions comprising a fibrous base incorporated in a composition 55 comprising a gelatinous material and casein.

5. A flexible projection screen resistant to atmospheric and climatic conditions comprising a fibrous base incorporated in a composition comprising gelatinous material, casein and cupric sulphate.

6. A projection screen resistant to atmospheric and climatic conditions comprising a fibrous base incorporated in a composition comprising 100 parts of glue, 208 parts of water, 10 parts of sodium fluoride, 100 parts

of glycerine and 80 parts of a composition comprising 100 parts of casein, 130 parts of water 12½ parts of borax and 1 part of cupric sulphate.

7. A projection screen comprising a body 70 including gelatinous material, glycerine and a liquid principally, and organic light-diffusing material together with a solvent therefor incorporated in said body.

8. A projection screen comprising a body 75 section formed principally from gelatine, material imparting flexibility to the completed screen and a liquid, and a light-filtering agent substantially uniformly incorporated in said body section.

9. A projection screen comprising a body section having a substantially inert light-diffusing agent and a light-filtering agent substantially uniformly incorporated therein.

10. A projection screen comprising a body 80 section having a light-diffusing agent, a light-filtering agent, and a germicidal agent substantially uniformly incorporated therein.

11. A projection screen containing gelatinous material, glycerine and a liquid principally, a light diffusing agent, a curing agent, a germicide, coloring material, and having a fibrous strengthening material incorporated therein, said light diffusing agent 85 being substantially uniformly incorporated in the other screen forming materials.

12. A projection screen composed of gelatinous material, glycerine and a liquid principally, casein, a ~~germicidal agent~~, an alkali, 100 a curing agent, coloring material, and having a sheet of fibrous material incorporated therein.

13. A projection screen composed of gelatinous material, glycerine, and a liquid principally, casein, sodium fluoride, borax, cupric sulphate, coloring material, and having a sheet of fibrous material incorporated therein.

In testimony whereof, we have affixed our 110 signatures to this specification.

ARTHUR C. PAYNE.  
DAVID F. NEWMAN.

115

120

125

130